

May 7, 1929.

T. R. DAVIS  
METHOD OF HARDENING BRAKE DRUMS OF MALLEABLE  
IRON DISK AUTOMOBILE WHEELS  
Filed May 17, 1926

1,711,835



Fig. 1



Fig. 3

Fig. 4

INVENTOR.  
Thomas R. Davis

BY

Chamberlain & Neumann  
ATTORNEYS.

Patented May 7, 1929.

1,711,835

# UNITED STATES PATENT OFFICE.

THOMAS R. DAVIS, OF FAIRFIELD, CONNECTICUT.

## METHOD OF HARDENING BRAKE DRUMS OF MALLEABLE-IRON DISK AUTOMOBILE WHEELS.

Application filed May 17, 1926. Serial No. 109,605.

This invention relates to improvements in the method of manufacturing malleable iron disk automobile wheels, and relates more particularly to the method of hardening the 5 brake drum portion of the wheel so as to insure it withstanding the required amount of wear to which it may be subjected.

By way of introduction I will first briefly review the method producing malleable iron, 10 to which my invention relates. Commercial malleable iron when cooling from the liquid state in which it is cast, and before the annealing process, is known as white iron. This iron has a characteristic silvery white 15 fracture and consists of an alloy of iron, carbon, silicon, manganese, sulphur and phosphorus. These elements are so proportioned that the casting as it cools contains no free carbon, that is all the carbon is combined with the iron as iron carbide and the resultant structure is a fairly homogeneous mixture of cementite and pearlite. The iron carbide of this mixture, however, is not in a stable condition, but under the influence 25 of a temperature in excess of the critical temperature, which for commercial white iron is about 1375 deg. Fah., extending over a number of hours will break down into its components of carbon and iron. This carbon, 30 however, which is precipitated from a solid structure does not have the facility of collecting together in large flakes or globules such as is characteristic of the carbon which is separated from a molten solution 35 and which is noticed in the fracture of gray iron. The carbon, or more properly graphite, which separates from the white iron when it is subjected to a heat in excess of its critical temperature and held for a number 40 of hours, is of a very finely pulverized condition and is scattered uniformly throughout the mass of the casting. The resultant structure may be considered as an extremely dense sponge with its pores filled 45 with temper carbon.

After the precipitation of carbon has been completed in the annealing furnace, commercial malleable iron is produced. The carbon in this state, that is temper carbon, 50 again is not stable when subject to high heat but, will go back into solution with the iron forming an iron carbide. The amount of the iron carbide or, in other words, the amount of carbon going into solution with 55 the iron, being in proportion to the tempera-

ture as the combination of carbon and iron with a rising temperature follows a definite curve. The combination of carbon and iron when malleable iron is heated, however, takes place almost instantaneously. I propose to take advantage of this phenomenon in case hardening the surface of the malleable iron brake drums as will later be more fully explained.

In the accompanying drawings:—

Fig. 1 shows a plan view of an apparatus by means of which my improved method of hardening the brake drums of cast metal wheels is carried out;

Fig. 2 is a cross sectional view, on a reduced scale, taken on line 2—2 of Fig. 1;

Fig. 3 shows a central vertical sectional view of a part of a malleable iron disk automobile wheel illustrating the original thickness of the brake drum; and

Fig. 4 shows a somewhat similar sectional view of a wheel, the brake drum being thinner than that shown in Figs. 1 and 3 having been turned down, and illustrating the application of heat to the inside of the brake drum instead of the outside as in Figs. 1 and 2.

In illustrating my invention I have shown a type of automobile wheel, covered by a recently obtained U. S. Letters Patent. 85 This wheel, as will be seen, is formed of a single malleable casting and includes a hub 6, an integral ribbed disk portion 7, an annular flange 8 and an integral annular cylindrical brake drum member 9. The wheel 90 is obviously formed of very thin, consequently relatively light, though strong malleable iron and in the usual manner of producing this kind of casting as hereinbefore set forth.

It is obviously important that the brake drum which, as before stated, is formed integral with the disk portion of the wheel, should first be made concentric with the axis of the wheel and secondly must be sufficiently hard to resist the extreme abrasion to which it is subjected by reason of the application of the brake. In the production of my wheel I therefore originally form the brake band portion of the wheel somewhat 105 thicker (as suggested by Fig. 3) than is actually necessary and turn the same down as at 10 either from the inside or outside according to which side the braking element is to be applied, said machining off 110

of the metal being preferably done after the wheel as a whole has been heat treated as in the art of making a malleable iron casting. This machining operation serves to remove the decarbonized skin of the brake drum and presents a surface that is impregnated with temper carbon which will be immediately combined with the iron with the application of heat in excess of the critical temperature, thus insuring a harder brake drum surface than would be possible to obtain with the decarbonized skin on the drum.

In the accompanying drawing I have shown a simple form of machine by means of which my invention may be carried out yet it will be obvious that other means or mechanisms may be employed to equally as good advantage and without departing from the spirit of the invention. I find that malleable iron automobile wheels of my improved type having integrally formed brake drums, can be best treated in accordance with my invention when mounted to rotate and by employing both heat and water as a means of hardening the brake drums. I have therefore devised a water tank 11 upon which is mounted a bearing 12 in which a portion of an arbor 13 is journaled to rotate. The outer end portion of said arbor is further journaled in a bearing 14 which may be secured to the floor, and the outer end of the arbor is provided with a pulley 15 by means of which the arbor and wheel may be rotated. The inner end of the arbor 13 is tapered as at 16, threaded and provided with a nut 17 for the detachable mounting of the malleable iron automobile wheel. The wheel may be thus mounted to be rotated while a horizontal jet of high temperature flame is placed against the side of the brake drum to be hardened, and during which time a spray of cold water is applied to the opposite side, and the lower portion 45 of the wheel rotated through the water tank 11.

As shown in Figs. 1 and 2, I have provided a horizontally disposed oxy-acetylene nozzle 18 in spaced relation to the outer peripheral surface of the brake drum, in position so that the flame therefrom will be directed across the width of the surface of the drum. This nozzle is mounted upon the inner end of a hollow arm 19 carried in a member 20 adjustably mounted in a standard 21 that is slidably mounted in a guideway 22 in which is positioned an adjusting screw 23 for moving the nozzle to and from the brake drum. The guideway 22 is mounted for pivotal adjustment upon a support 24 as at 25, and is provided with an adjusting screw 26 whereby the inner end of the said guideway and nozzle may be raised and lowered and best positioned with respect to the particular style and size of brake drum to

be hardened. The nozzle is provided with fuel supply pipes 27 and air pipes 28 whereby the required mixture of fuel may be provided. A water pipe 29 is also connected with the burner for cooling purposes.

For convenience of illustration, I have shown this pipe connected with the main water supply pipe 29 for the water nozzle 30 positioned within the brake drum and substantially opposite the position of the oxy-acetylene nozzle.

In Fig. 4 the relative positions of these two nozzles are reversed from that shown in Fig. 1, the oxy-acetylene nozzle being on the inside and the water nozzle being on the outside. By both of these arrangements the flame and water spray are directed against opposite sides of the brake drum just above the tank of water into which the wheel and drum revolves immediately upon leaving the flame.

The flame would not have time to heat more than just the surface of the metal before the metal would be plunged into the water and quenched. The water from the spray flows over the entire surface of the drum as it passes the flame and has the effect of always keeping one side of the drum opposite the flame from a dangerous heat. This prevents any warping of the drum and is an insurance against the drum becoming heated throughout in any one spot above the critical temperature, causing a plane of brittleness.

The flame itself could be directed directly against the surface of the drum, or it might be directed down or perhaps upward. The principle of the invention would be the same in all cases—that is, the surface of the drum would be flashed above its critical temperature while the back of the drum would be held to normal by application of water. This gives a very hard surface to the drum which we can regulate to any depth desired by the amount of heat applied and the amount of time that this application will last. At the same time, we maintain the body of the drum in the same strong malleable condition as when it came from the annealing furnace.

Having thus described my invention, what I claim and desire to obtain by Letters Patent is:

The herein described method of manufacturing a malleable iron automobile wheel, including a brake drum, which consists in machining off the outer periphery of the drum to remove the decarbonized skin of the brake drum and comprising a surface that is impregnated with temper carbon which will be immediately combined with the iron with the application of heat in excess of the critical temperature, directing a flame across the entire width of the outer periphery of the drum heating the machined

surface to a temperature in excess of the critical temperature while the drum is rotating, and simultaneously directing a spray of water across the entire width of the inner 5 periphery of the drum directly opposite the point of application of heat to maintain the inner periphery opposite the flame from a dangerous temperature, and maintain the in-

ner periphery of the drum at a temperature less than the critical temperature to prevent 10 warping of the drum.

Signed at Bridgeport in the county of Fairfield and State of Connecticut this 14th day of May, A. D. 1926.

THOMAS R. DAVIS.